# EUROPEAN PATENT SPECIFICATION

(11) **EP 0 045 828 B1**
(45) Date of publication and mention of the grant of the patent: **28.08.1985**
(21) Application number: 80830063.6
(22) Date of filing: 04.08.1980
(51) Int. Cl.: B27K 3/15

(54) **Improvement of the impregnation process of wood and other materials, with resins**
Verfahren zum Imprägnieren von Holz und anderen Materialien mit Harzen
Procédé d'imprégnation de bois et d'autres matériaux utilisant des résines

(43) Date of publication of application: 17.02.1982
(73) Proprietor: SIMPLE S.r.l., Ceccano (Frosinone) (IT)
(72) Inventor: Malavasi, Alberto, Roma (IT); Rio, Alberto, Colleferro (Roma) (IT)
(74) Representative: Mascioli, Alessandro, Prof.Dr.

## Description

As is already well known, certain procedures aim to improve the properties and the possible applications of various materials, based in their impregnation with resins. These processes generally involve the introduction of liquid organic monomers in the materials to be treated, followed by polymerization in situ, to prepare a composition material of higher quality.

Wood is one of the materials best suited to this treatment. As a construction material, wood exhibits striking defects arising from its structure and characteristics which limit and affect its applications.

These negative properties include its accentuated anisotropy, its permeability, its sensitivity to the action of aggressive atmospheric, biological and chemical agents, as well as its consequent rapid deterioration. The above are only attenuated with conventional protection systems based essentially on varnishing. Of all procedures designed to improve and broaden the range of application of wood, the most radical and sure solution is without doubt its impregnation with resins. This process has been used successfully particularly in the United States, where the wood is impregnated with organic monomers which are then polymerized, usually by radiation.

In addition to wood, there are many other materials which might be impregnated with resins, since this procedure can substantially improve their properties and broaden the range of their applications. These include cement mixtures, tiles and all materials with a porous structure. The elimination of this porosity causes a striking improvement in properties and application characteristics.

As mentioned above, the impregnation process is performed in two distinct phases.

In the first phase, after the material is dried and degassed, the monomer or mixture of monomers penetrates the cavities and capillaries in the material by means of capillary action, eventually assisted by pressure exerted by an inert gas like nitrogen.

The second phase involves the subsequent polymerization of the impregnating monomer or monomers. Solidifying in situ, the latter form a three-dimensional network in the structure of the material which eliminates most of the empty spaces.

Since the technique of radiation polymerization requires complex high investment installations and is quite dangerous, it has been replaced by thermo-catalytic-treatment which is simpler, more economical and risk-free. However, thermo- catalytic treatment also has considerable disadvantages, arising mainly from the use of chemical initiator or catalyst and heat. The monomer, in fact, becomes unstable once the catalyst has been added and therefore must be maintained constantly at a low enough temperature to prevent polymerization during the first phase of the precedure.

Another problem of greater importance, due to the difficulty of eliminating it, arises from the fact that thermocatalytic polymerization occurs with a highly exothermal reaction. During the reaction, the temperature increases sufficiently to cause, especially in wood, macroscopic phenomena of distortion as well as the formation of cracks and fissures due to the evaporation of the water still in the wood at the time of treatment. These distortions and cracks make the impregnated product completely unusable.

The excessive temperature increase further causes, due to the tendency of the monomer to evaporate before the transformation thereof into a polymer, the forming of a non compact, porous or even foamy polymer.

The present invention has the purpose of completely eliminating the problems mentioned above while at the same time perfecting the entire impregnation cycle by using for all phases of the process a single thermally regulatable and constant pressure apparatus or autoclave.

Thermo-catalytic treatments for the impregnation with resins are already well-known, but are substantially different from the object of the present invention.

In Patent FR-A-24 16 875 the wood, impregnated with acrilate, is immersed in water or other liquid for polymerization, and there does not exist any other temperature regulating system.

In Patent US-A-3 968 318 there is no temperature regulating system provided.

In Patent GB-1229700 the working cycle doesn't take place under constant pressure, but the material must be transferred from the impregnation container into the polymerization one.

The impregnation system covered by this invention is held to be simpler, must faster, more economical, and safer than the other systems currently available. In particular, with this system the exothermal polymerization reaction can be perfectly controlled. By perfectly graduating said reaction, this system allows the treatment of large quantities of material in a very short time, to give a product of higher technical and aesthetic quality.

The attached drawings, figures 1 to 8, show an illustrative and schematic representation of the various operations in the impregnation process, as described below.

In figure 1, the autoclave is charged with the material to be treated. Once it is closed, the cycle articulated in the various phases shown in figures 2, 3, 4, 5, 6 and 7 is begun. The autoclave is reopened when the cycle is completed (figure 8), and the finished product is removed.
A) In figure 1, the suitably dried material (2A) is introduced into the autoclave (1) using a container or cage. The material will be arranged so that the impregnating liquid can come in contact with all the surfaced to be treated, preventing the various pieces from sticking to one another during the polymerization phase.
B) In figure 2, the next operation, de-gassing, is represented. The air, represented by the dotted part (3), is removed through the tube (3A). De-gassing occurs at a residual pressure of 1.33xlO-³ bar to 66 to 10-³ bar for a total duration of 20 to 180 minutes.
C) As shown in figure 3, the autoclave is then filled with the monomer or mixture of monomers treated with the reaction catalyst. The monomer, represented by the wavy lines (4), is introduced through tube (4A). Said monomer can be easily introduced by utilizing the pressure difference between the supply reservoir and the autoclave. A cooling system which may, for example, involve the circulation of cold water or other refrigerant in the external jacket (5) of the autoclave (1), serves when necessary to keep the internal temperature at a safe level to prevent uncontrolled block polymerization of the monomer.
D) As shown in figure 4, once it has been filled so that the material is completely immersed in the monomer, the autoclave is pressurized with an inert gas, such as nitrogen. The monomer is indicated with (4), and the inert gas with the dots (6), introduced under pressure through tube (6A).
   Impregnation takes place at ambient temperature, preferably not above 20°C, to avoid the dangers of premature polymerization. To this end, the cooling system described (5) may be used. Impregnation takes place under a pressure of 1 to 10 bar of inert gas, for a total duration of 30 to 360 minutes.
E) As shown in figure 5, once impregnation has been effected, the residual monomer (4) is removed from the autoclave through tube (4B) while the inert gas atmosphere is maintained through tube (6A). Said monomer can be easily removed from the autoclave by utilizing the pressure difference between the autoclave and the monomer reservoir.
F) The thermocatalytic polymerization reaction is then initiated by raising the temperature inside the autoclave (see figure 6). While the heating may be effected-by circulating hot water or diathermal liquid in the external jacket of the autoclave, the main procedure used for heating involves injecting hot nitrogen in the autoclave to replace an analogous quantity of cold nitrogen forced out. The polymerization process initiated in this way occurs at a pressure equal to that used in the impregnation phase, at a temperature between 60° and 120° for a duration of 30-180 minutes.
G) The phase following initiation of the polymerization process is illustrated in figure 7. The temperature inside the autoclave tends to increase due to the heat generated by the exothermal polymerization reaction. It may be regulated with three different systems, used contemporaneously or individually as needed.

The first system involves circulating a refrigerant in the external jacket (5) of the autoclave, as already described at points C and D.

The second system uses de-gassing of the hot inert gas, necessary for keeping the pressure inside the autoclave constant. This pressure tends to increase as the temperature rises. This de- gassing is effected with the calibrated valve (7).

The third regulation system consists of inserting cold inert gas through tube (6A), keeping the pressure inside the autoclave constant. In this way, the hot output gas is relaced by the cold input gas (6A).

H) As shown in figure 8, once the reaction is completed as described, the treated material (2B) is removed from the autoclave after it has been returned to atmospheric pressure. It is now ready for use.

The drawings in figures 1 to 8 thus schematically represent the various phases of the process, which take place one after the other in the same apparatus or autoclave. As shown, except for the de-gassing, all the phases occur under constant pressure, including impregnation. In particular, an absolutely original part of this invention is the possibility of adjusting and regulating at will the internal temperature of the autoclave using the various systems cited above. There are: a) the outer jacket, which has the additional purpose during the impregnation phase of keeping the temperature inside the autoclave low enough to prevent block polymerization of the monomer; b) the regulation system involving what may be called dynamic control of the pressure, in which the pressure, which tends to rise as the temperature increases, is held constant through de-gassing and thus automatically decreases the temperature itself; c) the circulation, always under the same pressure, of a thermally adjustable and thermostatable fluid consisting of an inert gas, such as nitrogen.

The latter system is of particular importance to this invention. In fact, the gas, heated by a suitable external heat exchanger, is first circulated under pressure inside the autoclave at a temperature sufficient to heat the impregnated materials to be treated inside the autoclave. These materials are thus brought to the temperature at which the polymerization reaction initiates. Then, after the reaction has begun, the same gas, cooled by an external heat exchanger, is circulated under the same pressure to disperse the considerable heat of reaction. If uncontrolled, this heat of reaction would increase the temperature too much, causing great damages to the impregnated wood.

Therefore, nitrogen at constant. pressure and adjustable temperature is circulated within the container in order to: 1) keep the impregnating liquid inside the pores of the wood; preventing its leakage before polymerization; 2) first, bring the system of monomers to the reaction temperature and second, to disperse the excess heat from the highly exothermal polymerization reaction; 3) prevent the loss of evaporation of the water in the wood, and so maintain its original moisture level; 4) prevent the temperature from excessively increasing and thus causing in the impregnated wood a local evaporation, exudation and removing of the monomer, and a thermic bleaching.

As specified in this patent, said circulation is effected by inserting hot nitrogen for heating to replace an analogous quantity of cold output nitrogen and cold nitrogen for cooling to replace an analogous quantity of hot output nitrogen. The pressure inside the autoclave is always held constant.

The fundamental concept of this invention is thus the regulation of the temperature within the autoclave. In this regard, note that the condition for a good result from a process of impregnation followed by thermocatalytic polymerization is that the cooling be regulated perfectly during the exothermal reaction, so that the temperature inside the autoclave is always suitable for the treated material. In this regard, as a significant and original part of this invention which distinguishes it clearly from all others, the temperature inside the autoclave can be regulated perfectly using the various systems described. That is, a "thermally regulatable container or autoclave" is used.

### Examples

Examples of impregnating wood of diverse qualities:
1. Wood impregnated:
   Douglass, dried at 40°C for 24h. Impregnating system: Operating modalities:
      a) Impregnation:
      b) Polymerization: Impregnated resin: 58% by weight
2. Wood impregnated: Ramino, dried at 50°C for 48 h Impregnating system: Operating modalities:
   a) Impregnation:

   b) Polymerization: Impregnated resin: 48% by weight
3. Wood impregnated: European oak, dried at 50°C for 72 h Impregnating system: Operating modalities:
   a) Impregnation:

   b) Polymerization: Impregnated resin: 55% by weight

## Claims

1. Procedure for the impregnation of wood, wherein both the impregnation and the subsequent thermo-catalytic polymerization take place under pressure in a container or autoclave, wherein the pressure after degassing is always held constant in the various phases and a thermo- regulating autoclave is used, said autoclave allowing perfect regulation of the temperature in the various phases of the procedure, and wherein cooling of the monomer treated with reaction catalyst during the impregnation phase is effected by circulation of a fluid refrigerant in the outer jacket of the autoclave, so as to prevent the premature block polymerization of the monomer, and wherein the heating necessary to bring the impregnated materials inside the autoclave to the polymerization temperature is effected both by the circulation of a hot fluid in the outer jacket of the autoclave and, principally, by the insertion of hot nitrogen to replace an analogous quantity of cold output nitrogen, and wherein the heat arising from the exothermicity of the polymerization reaction is dispersed by the circulation of a fluid refrigerant in the outer jacket of the autoclave, and wherein the heat arising from the exothermicity of the polymerization reaction is dispersed by the de-gassing consequent to maintaining constant pressure inside the autoclave, and wherein the heat arising from the exothermicity of the polymerization reaction is dispersed by the insertion of cold nitrogen to replace an analogous quantity of hot output nitrogen.

2. Procedure as claimed in claim 1, wherein its use may be extended from wood to other impregnable materials with no modification, such as cement mixtures, tiles, metal alloy containers, and to any other suitable material.

## Patentansprüche

1. Verfahren zum Imprägnieren von Holz, wobei die Imprägnierung und die nachfolgende thermokatalytische Polymerisation unter Druck in einem Behälter oder Autoklav stattfindet, dadurch gekennzeichnet, dass:
- der Druck nach der Entgasung, während der verschiedenen Phasen, immer konstant gehalten wird;
-ein wärmegulierbarer Autoklav zur Verwendung kommt, der es erlaubt, die Temperatur während der verschiedenen Phasen der Vorganges immer ganau zu regulieren;
- die Abkühlung des zusätzlichen Monomers des Reaktionskatalysators während der Imprägnierungsphase durch Zirkulation einer abkühlenden Flüssigkeit in der äusseren Umhüllung des Autoklavs erreicht wird, um somit die vollständige, vorzeitige Polymerisation des Monomers zu verhinder;
- die notwendige Erwärmung, um die im Autoklav enthaltenen, imprägnierten Materialien bis zur Polymerisationstemperatur zu bringen, durch Zirkulation einer warmen Flüssigkeit in der äusseren Umhüllung des Autoklavs und besonders durch Einführung von warmen Stickstoff in Ersetzung einer gleichen Menge kalten, austretenden Stickstoffs erreicht wird;
- die Beseitigung der Hitze, durch die exothermische Polymerisationsreaktion hervorgerufen, durch die Zirkulation einer abkülenden Flüssigkeit in der äusseren Umhüllung des Autoklavs erreicht wird;
- die Beseitung der Hitze, durch die exothermische Polymerisationsreaktion hervergerufen, durch Entgasung erreicht wird, bedingt durch die Erhlatung eines konstanten Druckes im Inneren des Autoklavs;
- die Beseitigung der Hitze, bedingt durch die exothermische Polymerisationsreaktion, durch Einführung von abgekühltem Stickstoff in Ersetzung einer gleichen Menge austretendem, warmen Stickstoff erreicht wird.

2. Verfahren nach Anspruch 1, dadurch gekennzeichnet, dass dieses Verfahren ausser bei Holz, ohne Abänderungen, auch bei anderen, imprägnierungsfähigen Materialien Verwendung finden kann, wie Zementkonglomerate, Ziegel, Behälter aus Metallegierungen und allen anderen Materialien, die zu diesem Zweck geeignet sind.

## Revendications

1. Procédé pour l'imprégnation du bois, dans lequel soit l'impréganation, soit la polymérisation thermo-catalytique succesive, ont lieu sous préssion dans un réservoir ou autoclave, caractérisé en ce que la pression, après le dégazage, est maintenue, dans les phases diverses, toujours constante et en ce qu'on utilise une autoclave thermiquement réglable, permettant de régler parfaitement la température pendant les diverses phases du procédé, et caractérisé en ce que le refroidissement du monomère additioné du catalyseur de réaction, pendant la phase d'imprégnation, est réalisé par la circulation d'un fluide rafraichissant dans la chemise extérieur de l'autoclave, pour empêcher la polymérisation anticipée en bloc du monomère, et caractérisé en ce que le chauffage nécessaire pour porter les matériaux imprégnés, disposés à l'intérieur de l'autoclave à la température de polymerisation est réalisée, soit par la circulation d'un fluid chaud dans la chemise extérieure de l'autoclave, soit, principalement, par l'introduction d'azote chaud, que remplace une quantité analogue d'azote froid en sortie, et caractérisé en ce que la suppression de la chaleur, due à la exothermicité de la réaction de polymérisation, se réalise par un dosage, conséquent au maintien constant de la pression à l'intérieur de l'autoclave, et caractérisé en ce que la perte de chaleur, due à la exothermicité de la réaction de polymérisation, se réalise en introduisant de l'azote refroidi, que remplace une quantité égale d'azote chaud en sortie.

2. Procédé suivant la revendication 1, caractérisé en ce que son emploi peut s'étendre, en dehors du bois, sans modification, à d'autres matériaux imprégnables, comme les conglomérés du ciment, la briqueterie, les réservoirs d'alois et autres matériaux aptes à ce but.
